

F. W. LYLE.  
ELECTRIC TERMINAL.

APPLICATION FILED OCT. 30, 1911.

1,060,989.

Patented May 6, 1913.

Fig. 1.



Fig. 2.



Witnesses:

George W. Tilden  
J. Ellis, Clerk.

Inventor:

Fred W. Lyle,  
by Albin S. Dan  
His Attorney

# UNITED STATES PATENT OFFICE.

FRED W. LYLE, OF LYNN, MASSACHUSETTS, ASSIGNOR TO GENERAL ELECTRIC COMPANY, A CORPORATION OF NEW YORK.

## ELECTRIC TERMINAL.

1,060,989.

Specification of Letters Patent.

Patented May 6, 1913.

Application filed October 30, 1911. Serial No. 657,516.

To all whom it may concern:

Be it known that I, FRED W. LYLE, a citizen of the United States, residing at Lynn, county of Essex, State of Massachusetts, have invented certain new and useful Improvements in Electric Terminals, of which the following is a specification.

My invention relates to electrical resistance or similar units consisting largely or entirely of boron and has for its object the production of an effective current connection or terminal.

Electrical resistors consisting of elemental boron either alone or associated with certain other elements, such as carbon, have a very high negative temperature resistance coefficient which makes them very valuable. The quickness with which the resistor responds to changes of current increases rapidly with the temperature at which it is operated. It is desirable, therefore, to operate a resistor at high temperature when quick response is desired. In fact, even when not continually operating a boron resistor at high temperature, it is desirable to have the temperature range of its operation as wide as possible.

I have found that the metals of the chromium group particularly tungsten and molybdenum may be chemically united to boron articles so as to form unions of good mechanical strength and electrical conductivity and which will withstand high temperatures better than unions of boron and other metals, even others which are highly refractory. The boron article and the metallic terminal are heated while in contact by means of an external arc thereby causing chemical combination with the formation of a refractory alloy between the respective metal and the metalloid boron which unites the two into intimate conductive relation. It is important that the arc shall not be struck with either of the welded materials as this almost invariably produces over heating, and consequently cracking.

In the accompanying drawings, Figure 1 is an elevational view of an apparatus for fusing the cap or terminal to a boron resistor; Fig. 2 is an elevation taken at right angles to the view shown in Fig. 1 and Fig. 3 is a sectional detailed view of the boron resistor with the terminal applied.

The process of joining the terminal to the rod of boron is preferably carried out by heating the terminal and boron resistor

while in contact by means of an arc struck between two independent electrodes. This heating process is carried out in a reducing gas such as hydrogen, or in an inert atmosphere, in order to prevent the formation of oxids. Figs. 1 and 2 show the boron resistor 1 supported by long-handled tongs 2 within a bell jar 3. The bell jar is supplied with hydrogen or other suitable gas through a tube 4. As shown on the drawing, the tongs hold the boron rod in contact with the caps or terminals 5 by simple mechanical pressure. Carbon electrodes 6, 7 are held by suitable clamps on tongs 8, one member of which 9 is adjustable both vertically and horizontally by being pivoted on the insulating block 10. This block can be moved up and down the fixed rod which holds the electrode 6. Current is supplied by any suitable source of energy such as storage battery 11. An arc is struck by contact between the electrodes 6 and 7 and then gradually approached to the outside of the cap 5 which, as already mentioned, consists of tungsten, molybdenum or other metal of the same character. By gradually bringing the rod and terminal within effective heat-radiating distance of the arc, the weld is effected without cracking. The boron and the metallic cap are finally brought directly into the arc, thus completing the weld. The high temperature causes the boron and the metal of the terminal to chemically combine with the probable formation of an alloy which unites the rod and terminal into intimate conducting relation.

I have found tantalum to alloy with boron and to make a fairly good terminal, but the resulting alloy is somewhat brittle. I consider tungsten to be the most suitable metal for the purpose of my invention.

As shown in Fig. 3, I prefer to extend the metal cap 5 some distance outwardly from the end of the boron rod 1 to secure a certain amount of cooling effect at this region, and thus to enable suitable current connections to be made with convenience.

What I claim as new and desire to secure by Letters Patent of the United States, is,—

1. An electrical resistance consisting largely of elemental boron having a terminal consisting of a metal of the chromium group in intimate conducting relation thereto.

2. An electrical resistance composed

largely of boron and having a tungsten terminal welded thereto.

3. An electrical resistance composed of boron and having a tungsten terminal chemically united therewith.

4. An electrical resistance unit composed largely of boron, a terminal welded thereto consisting of a refractory material and an intermediate refractory alloy of said mate-

rial and boron integrally joining the terminal to the boron.

In witness whereof, I have hereunto set my hand this 26th day of October 1911.

FRED W. LYLE

Witnesses:

JOHN A. McMANUS, Jr.,  
FRANK G. HATTIE.